

## UNITED STATES PATENT OFFICE.

ROBERT JAY SHOEMAKER, OF CHICAGO, ILLINOIS, ASSIGNOR TO LEADIZING COMPANY, OF CHICAGO, ILLINOIS, A CORPORATION OF ILLINOIS.

## METAL-COATING PROCESS.

No Drawing. Original application filed April 15, 1920, Serial No. 374,089. Divided and this application filed July 18, 1920. Serial No. 397,179.

To all whom it may concern:

Be it known that I, ROBERT J. SHOEMAKER, a citizen of the United States, residing at Chicago, in the county of Cook and State of Illinois, have invented certain new and useful Improvements in Metal-Coating Processes, of which the following is a specification.

My invention relates to the operation of 10 coating or plating metal articles, such, for example, as articles of iron or steel, with a suitable plating metal such as lead or tin; and the primary object of the invention is to provide an improved plating process 15 which will be simpler and more economical than the processes heretofore used and whereby the article may be plated or coated with a film of the coating metal which will be very thin but at the same time even, 20 homogeneous and non-porous. The thinness of the plating makes it possible to plate articles such as threaded bolts, and the like, the threading of which, with ordinary methods, would be filled up by the plating metal. 25 Other incidental objects will be mentioned in connection with the following description of preferred methods of operation involving the principles of the invention.

A mixture is made of 50% or more of a 30 chloride of the plating metal, tin or lead, and 50% or less of zinc chloride. This mixture is heated to a temperature of about 600° Fahrenheit which produces a dissolving of the chlorides together and a disassociation of 35 the tin or lead chloride. The article to be plated is immersed in this solution, or if the article is hollow, the solution or its ingredients may be placed and heated in such hollow article. The tin or lead from the decomposed 40 tin or lead chloride deposits on the surface with which the molten solution comes into contact, forming a thin, homogeneous, non-porous and very adherent coating or plating. The chemical action is one 45 of substitution, iron from the article treated displacing the lead or tin in the chloride because of the greater affinity of the iron for the chlorine molecule in the sense of the following equation (assuming a lead plating operation)  $PbCl_2 + Fe = FeCl_2 + Pb$ . The zinc chloride does not enter into the reaction. In 50 lead plating the zinc chloride reduces materially the melting point of the solution,

which is an advantage as the melting point of lead chloride is very high. In the case 55 of a tin plating operation the zinc chloride keeps the solution from volatilizing. When the article is removed from the bath a certain amount of the tin or lead chloride will adhere to the article, which, because of its 60 insolubility, cannot be washed off as can the zinc chloride. The article is thereafter put into a vessel containing zinc chloride alone, 65 of the plating surface brought into contact with the zinc chloride, which is heated to approximately 600° Fahrenheit. The chloride of the plating metal will dissolve in the zinc chloride at that temperature, and when the article is taken from the bath the salt thus formed may be washed off with water. 70

By this method it is possible to plate the inside alone of an article such as a sheet metal can, boiler or a section of pipe. If the process is carried on by dipping the articles into a molten bath, the method has 75 the advantage over plating methods heretofore used that the articles may be handled a considerable number at a time instead of singly. The coating will be thinner and more even than that which results from the ordinary plating method, the metal will penetrate into small crevices, and, in general, 80 the plating will closely follow the surface of the article treated. Brass or copper articles may be plated by this method as well 85 as articles of iron or steel. In carrying out this process the amount of the chloride of the plating metal should not be substantially less than the amount of the zinc chloride. If it is substantially less the plating will not 90 be accomplished satisfactorily. This is due possibly to the solvent action of the zinc chloride upon the metal deposited. The method is suitable for plating billets for cold drawing or stamping in substitution 95 for the common method of "doping."

If iron or steel articles are plated with nickel or copper by the ordinary method of electrolysis, the iron or steel in time will 100 rust through the plating. This may be prevented by first coating the article according to the method above described with either tin or lead and then electroplating the article in the usual manner.

This application is a division of a prior 105 application filed April 15, 1920, Serial No.

374,089 (patented January 31, 1922 as No. 1,405,167).

I claim:

1. Method of plating a metal article with lead or tin which consists in subjecting the surface to be plated to contact with a molten bath containing a chloride of the plating metal capable of reacting with the metal to be plated to form a chloride of said metal to be plated and to produce deposition on said surface of a thin, dense, adherent film of the plating metal, then bringing the plated surface into contact with a solvent of the salt of the plating metal, at fusion temperature, and washing the article.
2. Method of plating an iron or steel article with a thin, adherent rust-proof film which consists in subjecting the surface to be plated to contact with a chloride of the plating metal and zinc chloride heated to

fusion to produce substitution in the first named chloride of the plating for the plating metal and deposition of the plating metal on said surface, then bringing the plated surface into contact with the zinc 25 chloride at fusing temperature to dissolve the adherent chloride of the plating metal.

3. Method of plating a metal article which consists in bringing the surface to be plated into contact with a chloride of the plating 30 metal and zinc chloride at a temperature of substantially 600° Fahrenheit to produce disassociation of the chloride of the plating metal and deposition of the plating metal on said surface, then bringing said plated surface into contact with zinc chloride heated to a temperature of substantially 600° 35 Fahrenheit, and washing to remove the adherent salt.

ROBERT JAY SHOEMAKER.

374,089 (patented January 31, 1922 as No. 1,405,167).

I claim:

1. Method of plating a metal article with lead or tin which consists in subjecting the surface to be plated to contact with a molten bath containing a chloride of the plating metal capable of reacting with the metal to be plated to form a chloride of said metal to be plated and to produce deposition on said surface of a thin, dense, adherent film of the plating metal, then bringing the plated surface into contact with a solvent of the salt of the plating metal, at fusion 10 temperature, and washing the article.
2. Method of plating an iron or steel article with a thin, adherent rust-proof film which consists in subjecting the surface to be plated to contact with a chloride of the plating metal and zinc chloride heated to 20
3. Method of plating a metal article which consists in bringing the surface to be plated into contact with a chloride of the plating metal and zinc chloride at a temperature of substantially 600° Fahrenheit to produce disassociation of the chloride of the plating metal and deposition of the plating metal on said surface, then bringing said plated surface into contact with zinc chloride heated to a temperature of substantially 600° Fahrenheit, and washing to remove the adherent salt.

ROBERT JAY SHOEMAKER.

#### Certificate of Correction.

It is hereby certified that in Letters Patent No. 1,533,473, granted April 14, 1925, upon the application of Robert Jay Shoemaker, of Chicago, Illinois, for an improvement in "Metal-Coating Processes," an error appears in the printed specification requiring correction as follows: Page 1, line 97, beginning with the word "If" strike out all to and through the word "manner", line 104; and that the said Letters Patent should be read with this correction therein that the same may conform to the record of the case in the Patent Office.

Signed and sealed this 23d day of June, A. D. 1925.

[SEAL.]

KARL FENNING,  
Acting Commissioner of Patents.

**Certificate of Correction.**

It is hereby certified that in Letters Patent No. 1,533,473, granted April 14, 1925, upon the application of Robert Jay Shoemaker, of Chicago, Illinois, for an improvement in "Metal-Coating Processes," an error appears in the printed specification requiring correction as follows: Page 1, line 97, beginning with the word "If" strike out all to and through the word "manner", line 104; and that the said Letters Patent should be read with this correction therein that the same may conform to the record of the case in the Patent Office.

Signed and sealed this 23d day of June, A. D. 1925.

[SEAL.]

**KARL FENNING,**  
*Acting Commissioner of Patents.*